

W. W. KIRBY.  
PROCESS OF FORMING PRINTING PLATES.  
APPLICATION FILED OCT. 28, 1915.

1,219,332.

Patented Mar. 13, 1917.

Fig. 1.



Fig. 2.



<sup>Inventor</sup>  
Wallace W. Kirby

Witnesses

Albert P. Hopkins  
Grace P. Brewster

By

Stewart & Mason

Attorneys

# UNITED STATES PATENT OFFICE.

WALLACE W. KIRBY, OF WASHINGTON, DISTRICT OF COLUMBIA, ASSIGNEE, BY MESNE ASSIGNMENTS, TO THE RAPID PROCESS LITHOGRAPH COMPANY, INC., A CORPORATION OF DELAWARE.

## PROCESS OF FORMING PRINTING-PLATES.

1,219,332.

Specification of Letters Patent. Patented Mar. 13, 1917.

Application filed October 28, 1915. Serial No. 58,443.

*To all whom it may concern:*

Be it known that I, WALLACE W. KIRBY, a citizen of the United States, residing at Washington, in the District of Columbia, have invented certain new and useful Improvements in Processes of Forming Printing-Plates, of which the following is a description.

The invention relates to new and useful improvements in the process of making printing plates, and more particularly a metal printing plate having a plane printing surface.

Prior to my invention, efforts have been made to produce a printing plate by coating the same with a sensitized film, exposing the same under the design to be reproduced and subsequently developing the design. Difficulties have been experienced, however, in obtaining a clear cut and well defined reproduction of the design on the plate.

An object of the present invention is to devise a process of treating the plate whereby the sensitized film may be removed from the plate and the non-printing surface finished, leaving a printing surface on the plate which is a clear cut and well defined reproduction of the original design.

Figure 1 is a sectional view through a plate having a sensitized film thereon; and

Fig. 2 is a view of the same after the unexposed portions have been washed out and the film treated to form a crust thereon.

The invention consists broadly in applying a suitable sensitized film to a metal plate, exposing said sensitized surface to light and washing out the unexposed portions covered by the design, subsequently treating the plate so as to thoroughly clean the printing surface of any possible traces of the film and also softening the film to facilitate its removal from the plate. After the film has been softened, the surface of the film is hardened or formed with a slight crust, over which is placed a coating of a fatty acid-resisting substance and then the plate is washed or otherwise subjected to a dilute acid treatment for removing the film. The plate is then finished in the usual manner, leaving a well defined reproduction of the design.

Referring more in detail to the invention: My improved process consists in prepar-

ing a grained metal plate 1 either of aluminum or zinc by applying thereto a sensitized film 2 which may be made of glue or any other suitable base mixed with ammonium bichromate, potassium bichromate, or any other suitable chemical which will produce sensitive film, capable of being rendered insoluble by light. This film is, of course, dried.

The design to be reproduced on the printing plate is made on a transparent sheet or substance by any suitable opaque liquid, and this original drawing is used direct in the production of the printing plate, thus eliminating the camera and negative. The original drawing or design is placed on the sensitized plate and exposed to light. The exposed parts of the film are rendered insoluble by the action of the light thereon, while the unexposed parts of the film beneath the design remain soluble and may be washed off by water after the exposure has been made. After the plate has been washed, I apply a dye, such as violet dye which is soluble in alcohol which causes the subject or design indicated at 3 in the drawing to appear very clearly, providing a proper exposure has been made.

No matter how carefully the plate may be washed, very often particles of the film will adhere to the printing surface, that is, the surface beneath the design which has not been exposed to the light; and in order that a clear cut, well-marked reproduction of the design may be made, it is essential that this printing surface should be thoroughly clean before the same is treated with a fatty acid-resisting substance. In order to accomplish this, I flow over the plate for a brief period of time a solution of potassium hydrate or the equivalent thereof. This solution of potassium hydrate thoroughly cleanses the printing surface and softens the film, which greatly facilitates the removal of the film at a later step in the process. After having subjected the plate to the solution of potassium hydrate treatment, I next apply alcohol until all the violet coloring leaves the plate. The primary purpose of the alcohol is to surface-harden or crust the softened film as indicated at 4 in Fig. 2 of the drawing so that a coating of an acid-resisting substance such as an asphaltum solution may be ap-

plied to the plate without said substance penetrating the film and adhering to the non-printing surface of the plate.

The plate is then dried and, when 5 thoroughly dry, an asphaltum solution is applied. This forms a thin even coating and is allowed to set or dry. The plate is then subjected to a hydrochloric acid solution and rubbed very lightly until the plate 10 is cleaned of all traces of the film and the design or subject stands out clearly. The plate is then washed to remove all traces of the acid. When the asphaltum coating is applied to the plate, it adheres very closely 15 to the cleaned printing surface and forms a thin coating over the film.

When the plate is subjected to the hydrochloric acid solution, the acid penetrates the relatively thin asphaltum coating on the 20 film and undercuts the film so that it may be readily removed, leaving the plate coated with the asphaltum solution only at the part or parts containing the design or subject. The plate is then finished in the manner well 25 known in this art.

From the above, it will be apparent that the three essential features of my invention consist: first, in the thorough cleansing of the printing surface corresponding to the 30 subject or design prior to the application of the acid-resisting substance thereto; second, the softening of the base or film prior to the applying of the asphaltum coating thereto so that the same may be subsequently readily 35 removed by the acid treatment; and third, surface-hardening of the film or forming a crust thereon so that the asphaltum solution may be applied in a thin coating thereon and kept away from the non-printing 40 surface of the plate. These three features contribute to the production of a printing plate having a plane surface thereon wherein the subject or design is clear cut and well defined.

45 It is obvious that minor changes in the details stated and in the specific chemicals used and in the order of applying the same may be made without departing from the spirit of the invention, as set forth in the 50 appended claims.

Having thus described my invention, what I claim as new and desire to secure by Letters Patent, is:—

1. The process of making a printing plate 55 which includes applying to a metal plate a sensitized film capable of being rendered insoluble by light, exposing the plate under the desired design, washing out the unexposed portions covered by the design, wash- 60 ing said plate with a solution to soften the film, hardening the surface of the film, coat-

ing the plate with an acid-resisting substance, and removing the film by an acid.

2. The process of making a printing plate which includes applying to a metal plate a 65 film capable of being rendered insoluble by light, exposing the plate under an original drawing of the desired design, washing out the unexposed portions beneath the design, washing said plate with a caustic alkaline 70 solution to soften the film and to clean the exposed printing surface of the metal, hardening the surface of the film, coating the plate with an acid-resisting substance, and removing the film by acid. 75

3. The process of making a printing plate which includes applying to a metal plate a sensitized film capable of being rendered insoluble by light, exposing the plate to a desired design, washing out the unexposed 80 portions beneath the design, washing said plate with a caustic alkaline solution to soften the film and to clean the exposed printing surface, washing said plate with alcohol to harden the surface of the film, 85 coating the film and printing surface with an acid-resisting substance, and subjecting the plate to a dilute acid solution to remove the film.

4. The process of making a printing plate 90 which includes applying to a metal plate a sensitized film capable of being rendered insoluble by light, exposing the plate under an original drawing of the desired design, washing out the unexposed portions beneath 95 the design, washing said plate with a solution of potassium hydrate, then washing said plate in alcohol, coating the film and printing surface with an asphaltum solution, subjecting said plate to a dilute hydro- 100 chloric acid to remove the film.

5. The process of making a printing plate which includes applying to a metal plate a sensitized film capable of being rendered insoluble by light, exposing the plate under an 105 original drawing of the desired design, washing out the unexposed portion beneath the design, applying to the film a dye, washing said plate with a solution which softens the film and cleanses the exposed printing surface of the metal printing plate, washing the plate with alcohol to remove the dye and to crust harden the film, coating the film and printing surface with an acid-resisting substance and finally subjecting the plate 110 to a dilute acid to remove the film. 115

In testimony whereof, I affix my signature in the presence of two witnesses.

WALLACE W. KIRBY.

Witnesses:

E. H. PARKINS,  
GRACE P. BRERETON.